

Nov. 12, 1929.

G. H. WILLIS

1,735,369

COMPOSITE RUBBER HEEL

Filed July 5, 1928

*Fig. 1*



*Fig. 2*



*Fig. 3*



Inventor  
Glenn H. Willis  
By Robert McPheron  
Atty.

## UNITED STATES PATENT OFFICE

GLENN H. WILLIS, OF AKRON, OHIO, ASSIGNOR TO JOHN L. SNYDER, OF AKRON, OHIO

## COMPOSITE-RUBBER HEEL

Application filed July 5, 1928. Serial No. 290,309.

This invention relates to rubber heels of the type employing a seating layer vulcanized to the heel body and strengthened with an intermixture of reinforcing material.

5 The use of embedded metallic washers for retaining the nail heads has heretofore been nearly universal, although inserts of wood have lately been used to some extent, thereby reducing the labor and material cost but giving a less flexible and resilient heel.

10 The object of my invention is to provide a heel of relatively-high flexibility and resiliency without the use of metallic washers and at a reduced labor cost. To this end I employ an attaching plug or layer inseparably bonded by vulcanization to the heel body, said layer being of leathery firmness, that is, sufficiently hard to retain the nail heads and counteract the spreading tendency of the 15 softer rubber of said heel body, but also possessing some resiliency which contributes to the cushioning properties and enough flexibility to produce a tight seating of the heel, especially at the edges.

20 25 I have found that these characteristics are obtained by incorporating in the rubber compound of the attaching plug or layer a reinforcement of grain hulls, the preferred material being oat hulls.

30 Of the accompanying drawings:

Fig. 1 is a top plan view of a rubber heel embodying my invention.

Fig. 2 is a perspective view of the attaching plug or layer.

35 Fig. 3 is a sectional view of a portion of a heel mold containing the heels, which are shown in transverse section.

In the drawings, 10 is the resilient heel body composed of suitable rubber compound 40 such as a good reclaimed rubber, with or without new rubber, and containing the usual pigments, sulphur for vulcanization and accelerator.

45 The attaching layer is a shallow inlay or plug 11 composed of rubber compound of about the same quality as the body compound, or it may be a cheaper quality, together with a reinforcement consisting of grain hulls 12 distributed throughout its mass. The best 50 hulls I have found for the purpose are oat

hulls which are relatively cheap and of high reinforcing value. Since they replace a considerable amount of the more expensive rubber material, their use effects some saving in the total cost of the heel. A large saving in 55 labor cost is of course also effected by dispensing with heel washers.

The proportion of oat hulls employed is approximately thirty percent of the total weight of the stock in the attaching layer, 60 but this proportion may be considerably varied. The rubber stock in the layer 11 is made relatively soft or sappy by the introduction of five to six percent of a flux or softener such as cottonseed oil, palm oil or 65 a suitable combination of vegetable and mineral oils in order to facilitate the distribution of the hulls throughout the plastic rubber. Milling is preferably performed on even-speed rolls having an open setting to 70 avoid a bank and the hulls are fed between the rolls into the sheet which follows one of the rolls, the opening being increased as the volume builds up.

75 When a homogeneous mixture has been obtained, the compound is run into a sheet of the desired thickness and flat blanks or plugs 11 of the shape shown in Fig. 2 are died out of said sheet. For each heel, one of these plugs is located in the cavity of a vulcanizing mold 13 to form an inlay on the attaching face of the heel and is retained in proper position by pins 14 on the lower mold plate. The body rubber being placed against the plug, the mold is then closed and the heel 80 vulcanized, both body rubber and plug being completely cured in the same period of time.

85 The labor cost for making heels with these attaching layers is less than for the common type having embedded washers and the results are superior. The layer 11 is readily penetrated by the nails but the nail heads are retained by this layer so that the heel may be firmly and durably secured on the shoe, the rubber in the attaching layer being present in 90 sufficient amount to form an inseparable vulcanized bond with that of the heel body. The resiliency of the inlay 11 contributes to the cushioning properties and its flexibility is such that a tight seating of the body rubber 95 100

around the edges is insured when the heel is nailed in place. The firmness of this inlay resists the tendency of the softer body rubber to spread substantially after the attachment has been effected.

5 The drawing illustrates a preferred form and arrangement of attaching layer reinforced as described but the details can be varied without departing from my invention.  
10 This idea may also, if desired, be utilized for attaching rubber soles to shoes.

I claim:

15 1. A composite, vulcanized rubber shoe tread which is flexible and resilient throughout, said tread comprising a rubber cushion wearing body, and an attaching layer of leathery firmness integrally vulcanized to said cushion body and formed of rubber intermixed with grain hulls, said layer being  
20 adapted to retain nail heads and resists the lateral spreading tendency of the cushion body.

25 2. A composite, vulcanized rubber heel comprising a rubber cushion body, and a flexible, resilient, attaching layer integrally united with and inlaid in the seating face of said body, said layer being composed of rubber compound containing grain hulls having substantially the stiffness of oat hulls.

30 3. A composite, vulcanized rubber heel comprising a rubber cushion body, and a flexible, resilient, attaching layer integrally united with and inlaid in the seating face of said body, said layer being composed of rubber compound containing a minor proportion  
35 of oat hulls.

In witness whereof I have hereunto set my hand this 29th day of June, 1928.

GLENN H. WILLIS.

40

45

50

55

60

65